# EUROPEAN PATENT SPECIFICATION

(11) **EP 0 048 579 B1**
(45) Date of publication and mention of the grant of the patent: **19.12.1984**
(21) Application number: 81304194.4
(22) Date of filing: 14.09.1981
(51) Int. Cl.: C25D 3/56, C25D 17/10, C25D 17/02, C25C 7/04

(54) **Method for the electro-deposition of lead alloys**
Verfahren zur galvanischen Abscheidung von Bleilegierungen
Procédé pour le dépôt électrolytique d'alliages de plomb

(30) Priority: 23.09.1980 GB 8030638
(43) Date of publication of application: 31.03.1982
(73) Proprietor: GKN VANDERVELL LIMITED, Maidenhead Berkshire SL6 4BG (GB)
(72) Inventor: Waterman, William John, Bourne End Bucks (GB); Brook, Miachel Gordon, Chessington Surrey (GB); Jenni, Lita Elizabeth, Maidenhead Berks (GB)
(74) Representative: Thorpe, Brian

## Description

This invention relates to a method for the electro-deposition of an alloy coating on to a backing member, such a process being of particular interest to the coating of a load carrying bearing surface on to the backing member of a plain bearing.

Such a bearing may comprise for example a half shell backing member of steel with a bronze substrate bonded thereto and on to which is electro-deposited a bearing surface coating of lead-indium or lead-antimony-tin. Binary and ternary alloys can be co-deposited electrolytically as is described for example in British Patents 577335 and 628459 and in U.S.A. Patent 2605149. In British Patents 577335 it is stated, and has been verified in tests, that coatings of ternary alloys such as lead-antimony-tin or lead-tin-copper can replace the more usual lead-tin or lead- indium binary alloy coatings as bearing surfaces.

However in the electro-deposition of ternary alloys containing antimony or copper, there is a displacement reaction when a soluble metal anode is used. For example in British Patent 628459 it is stated that antimony will immersion plate on to a lead, lead-tin or lead-tin- antimony anode. In Patent 628459 it is stated that this immersion plating is adherent enough so that the anode may be used two or three times and then the antimony may be scrubbed off and reclaimed and, whereas such a procedure may be acceptable for small scale operation, it would not be feasible to operate a continuous production plating process wherein anodes were required to be removed many times during the working operation for scrubbing.

Similarly if a lead-tin-copper electrolyte is utilised, the copper in the plating solution immersion plates out on to metal anodes such as lead or lead-tin and, although such an electrolyte has been in production used for many years, the removal of all the anodes from the bath during idle periods is required, and the frequent additions of copper fluoroborate are necessary to replace losses from the electrolyte.

It is the object of the present invention to provide an improved method which will prevent the undesirable immersion plating of a soluble metal anode containing lead by metals from the plating solution which are more noble then lead.

In accordance with the invention there is provided a method of electro-depositing a lead alloy onto a metal cathode characterised by the steps of immersing the cathode in a first chamber containing a lead based catholyte solution; immersing a soluble lead alloy anode in a second chamber containing a lead based anolyte solution which does not contain ions capable of immersion plating onto the anode; maintaining the anolyte solution and the catholyte solution separate from one another by the medium of a cation exchange membrane; and applying a direct current between the anode and the cathode.

It is preferred that the second chamber is located wholly within the first chamber.

In use of the method according to the invention the anolyte will not contain elements capable of immersion plating on to the anode. Thus if the catholyte comprises a lead-antimony-tin plating solution then the anolyte will not contain any antimony. Similarly if the catholyte comprises a lead-tin-copper plating solution then the anolyte will not contain copper.

According to the method of the invention, metal ions arising from the anode pass through the cation exchange membrane towards the cathode under the influence of the plating potential. Since the anolyte contains no metal capable of immersion plating on to the anode will remain clean. At the end of the plating operation, when the plating potential is disconnected, the animony or copper or arsenic in the catholyte (depending on what alloy is being co-deposited) is prevented from entering the anolyte by the physical barrier of the cation exchange membrane. That is to say, metal ions can pass in one direction only, i.e. towards the cathode, and then only under the influence of the plating potential applied between the anode and cathode. Thus the anolyte solution in the second chamber remains free of ions capable of immersion plating on to the anode.

A further advantage of the use of a cation exchange membrane to physically separate the catholyte and anolyte solutions is that the composition of the catholyte may be controlled more readily since metal is not lost therefrom by immersion plating which in turn means that the electro-deposited alloys have more consistent compositions.

Other features of the invention will become apparent from the following description given herein solely by way of example and with reference to the accompanying drawing which shows, in diagrammatic form, a plan view of a plating apparatus for use in the process in accordance with the invention.

Referring to the drawings, there is shown a first chamber 10 within which is locatable a member 12 to be plated and which comprises the cathode; such member may comprise a steel backing member with a bronze substrate bonded thereto and on to which is to be co-deposited a ternary alloy as a bearing surface. This first chamber 10 is capable of being filled with the catholyte solution.

At the end of the first chamber 10 remote from the cathode 12 there is provided a second chamber 14 wholely contained within the first chamber and communicating therewith only through the medium of a cation exchange membrane 16. This second chamber 14 is conveniently of box like rectangular configuration having an open top and an open front across which is secured the exchange membrane 16 by means of detachable clamping plates and gaskets. To provide support and protection for the exchange membrane 16 a sheet 18 of porous polyethylene may be sealingly located by the gaskets on one or both sides of the membrane 16 the polyethylene sheeting 18 being provided to prevent physical damage to the exchange membrane 16 and also providing support against sag or swelling of the exchange membrane which may occur in use.

The cation exchange membrane is a proprietary item and may be of the type available from Permutit-Body of Brentford, Middlesex, England.

The anode 20 is locatable within the second chamber 14 and the chamber 14 is capable of being filled with an anolyte solution to at least the same level as that of the catholyte solution in the first chamber 10. It may be preferable for the level of the anolyte solution to be above that of the catholyte solution to provide a slight hydrostatic pressure in favour of the anolyte.

The following examples of use of the apparatus will serve to illustrate the invention:-

### Example 1

The apparatus was used for the electro-deposition of a ternary alloy of lead-antimony-tin to give a coating having a basis of lead and containing between 9.5% and 10.5% by weight of antimony and between 5.5% and 6.5% by weight of tin in the deposited alloy. The anode was a lead-tin anode containing 5% to 25% by weight of tin.

The cathode comprised a steel backing member on to which was bonded a bronze substrate. It is preferable to electroplate a base coating of cobalt or nickel on to the bronze substrate thereby to give a better surface for the deposition of the required ternary alloy particularly for the prevention of dispersal of tin into the bronze.

The catholyte solution in the first chamber was as follows:-

The temperature of the catholyte was maintained at 40°C and a cathode current density of 30 amperes per square foot was utilised for approximately 20 minutes to give a deposited alloy thickness of 25 um.

The second chamber was filled with an anolyte solution of the following composition

The temperature of the anolyte solution was maintained at 40°C

### Example 2

In this example identical constructions of anode and cathode were utilised as in the preceding example but the electrolyte solutions were chosen to give a ternary alloy deposit on the cathode of lead-tin-copper having a basis of lead and containing between 8% and 12% of weight of tin and between 2% and 3% by weight of copper in the deposited alloy.

A catholyte solution of the following compositions was used:

The temperature of the catholyte solution was maintained at 25°C and cathode current density of 20 amperes per square foot was utilised for approximately 20 minutes to give a deposited ternary alloy of 25,um thickness.

The anolyte solution was identical in all respects with the catholyte solution with the exception that no copper fluoroborate was present in the anolyte.

In both examples it was found that the anode remained clean and that the plating elements had been lost from the catholyte to the cathode at a controlled rate.

## Claims

1. A method of electro-depositing a lead alloy onto a metal cathode (12) characterised by the steps of immersing the cathode (12) in a first chamber (10) containing a lead based catholyte solution; immersing a soluble lead alloy anode (20) in a second chamber (14) containing a lead based anolyte solution which does not contain ions capable of immersion plating onto the anode; maintaining the anolyte solution and the catholyte solution separate from one another by the medium of a cation exchange membrane (16); and applying a direct current between the anode and the cathode.

2. A method according to Claim 1 further characterised in that the catholyte solution is a lead-antimony-tin solution, the anolyte solution is a lead-tin solution and the anode (20) is a lead-tin anode.

3. A method as claimed in Claim 1 further characterised in that the catholyte solution is a lead-tin-copper solution, the anolyte solution is a lead-tin solution and the anode (20) is a lead-tin anode.

4. A method according to any one of the preceding claims further characterised in that the second chamber (14) is located wholly within the first chamber (10).

5. A method according to any one of the preceding claims further characterised in that the cathode (12) is a steel backed bearing member.

## Patentansprüche

1. Verfahren zur galvanischen Abscheidung von Bleilegierungen auf einer Metallkathode (12), dadurch gekennzeichnet, daß die Kathode (12) in eine erste, eine auf Blei basierende Katholytlösung enthaltende Kammer (10) eingetaucht wird, daß eine aus einer löslichen Bleilegierung bestehende Anode (20) in eine zweite Kammer (14) eingetaucht wird, die eine auf Blei basierende Anolytlösung enthält, die keine Ionen enthält, die auf der Anode stromlos einen Überzug bilden können, daß die Anolytlösung und die Katholytlösung mittels einer Kationaustauschmembran (16) voneinander getrennt sind und daß zwischen die Anode und Kathode Gleichstrom eingeführt wird.

2. Verfahren nach Anspruch 1, dadurch gekennzeichnet, daß es sich bei der Katholytlösung um eine Blei-Antimon-Zinn-Lösung, bei der Anolytlösung um eine Blei-Zinn-Lösung und bei der Anode (20) um eine Blei-Zinn-Anode handelt.

3. Verfahren nach Anspruch 1, dadurch gekennzeichnet, daß die Katholytlösung eine Blei-Zinn-Kupfer-Lösung, die Anolytlösung eine Blei-Zinn-Lösung und die Anode (20) eine Blei-Zinn-Anode ist.

4. Verfahren nach einem der vorhergehenden Ansprüche, dadurch gekennzeichnet, daß die zweite Kammer (14) sich vollkommen innerhalb der ersten Kammer (10) befindet.

5. Verfahren nach einem der vorgergehenden Ansprüche, dadurch gekennzeichnet, daß es sich bei der Kathode (12) um einen durch Stahl verstärkten Lagerkörper handelt.

## Revendications

1. Un procédé de dépôt électrolytique d'un alliage de plomb sur une cathode métallique (12) caractérisé par les phases consistant à immerger la cathode (12) dans une première chambre (10) qui contient une solution catholyte à base de plomb; immerger une anode soluble (20) en alliage de plomb dans une deuxième chambre (14) contenant une solution anolyte à base de plomb qui ne contient pas d'ions capables de se déposer en immersion sur l'anode; maintenir la solution anolyte et la solution catholyte séparées l'une de l'autre au moyen d'une membrane échangeuse de cations (16); et appliquer un courant continu entre l'anode et la cathode.

2. Une procédé selon la revendication 1, caractérisé en ce que la solution catholyte est une solution plomb-antimoine-étain, la solution anolyte est une solution plomb-étain et l'anode (20) est une anode plomb-étain.

3. Un procédé comme revendiqué dans la revendication 1, caractérisé en outre en ce que la solution catholyte est une solution plomb-étain-cuivre, la solution anolyte est une solution plomb-étain et l'anode (20 est une anode plomb-étain.

4. Un procédé selon l'une quelconque des revendications précédentes, caractérisé en outre en ce que la deuxième chambre (14) est entièrement logée dans la première chambre (10).

5. Un procédé selon l'une quelconque des revendications précédentes, caractérisé en outre en ce que la cathode (12) est un élément de palier à support d'acier.
